

## UNITED STATES PATENT OFFICE

2,303,404

## ALLOY

Cecil Spencer Sivil, Roselle, N. J., assignor to  
Baker & Company, Inc., Newark, N. J., a corpo-  
ration of New Jersey

No Drawing. Application December 20, 1941,  
Serial No. 423,793

## 3 Claims. (Cl. 75—172)

This invention relates to alloys and is con-  
cerned in particular with platinum metal alloys.

It is one object of my invention to provide al-  
loys of great corrosion resistance, high melting  
point and great hardness and strength. It is  
another object of my invention to provide such  
alloys of great electrical resistance. It is a fur-  
ther object of my invention to provide such alloys  
of low specific gravity and low cost.

This application is a continuation in part of  
my application Serial No. 401,653 filed July 9,  
1941, which in turn is a continuation in part of  
my application Serial No. 378,376, filed February  
11, 1941.

The alloys according to my invention com-  
prise palladium, ruthenium, and iridium. In  
such alloys the palladium content may be as  
low as about 60% and as high as about 95%, the  
ruthenium content being as low as 0.5% and as  
high as about 20%, whereas the iridium content  
comprises at least 2.5% of the whole alloy. I  
prefer alloys wherein the ruthenium content lies  
between about 1% and a maximum of about  
10%. In its best embodiments the alloys consist  
entirely of palladium, ruthenium, and iridium  
in the proportions specified herein, although, of  
course, minor quantities of other metals may  
be present so long as they do not substantially  
affect the beneficial properties and characteris-  
tics of my alloys.

Particularly advantageous are alloys within the  
limits of 80% to 96.5% palladium, 1% to 10%  
ruthenium, and 2.5% to 10% iridium, such as

alloys of 80% palladium 10% ruthenium and 10%  
iridium, or of 90% palladium 5% ruthenium  
and 5% iridium. Likewise, alloys comprising pal-  
ladium, ruthenium and iridium, according to my  
invention, may also contain advantageously a  
substantial content of rhodium, such as from  
2.5% to 37% rhodium, in which case the maxi-  
mum palladium content will be 94.5% and the  
maximum iridium content will be 37%, such as  
alloys of 80% palladium 5% ruthenium 5% iri-  
dium and 10% rhodium, or of 90% palladium  
2.5% ruthenium 2.5% iridium and 5% rhodium.  
In order to illustrate the properties of the al-  
loys according to this invention, I may state that  
an alloy of 80% palladium 5% ruthenium 10%  
rhodium and 5% iridium has a tensile strength  
of 133,900 lbs. per square inch when hard, and  
of 94,200 lbs. per square inch when annealed,  
and an elongation of 27% on 2-inches when an-  
nealed. The alloy, likewise, possesses an elec-  
trical resistivity of 200 ohms/mil ft.

What I claim is:

1. An alloy of palladium, ruthenium and iri-  
dium comprising 60% to about 95% palladium,  
0.5% to 20% ruthenium, and 2.5% to 39.5%  
iridium.
2. An alloy of palladium, ruthenium and iri-  
dium comprising 80% to 96.5% palladium, 1%  
to 10% ruthenium, and 2.5% to 10% iridium.
3. An alloy of palladium, ruthenium and iri-  
dium comprising about 90% palladium, about 5%  
ruthenium, and about 5% iridium.

CECIL S. SIVIL.